

## UNITED STATES PATENT OFFICE.

JUDSON A. DE CEW, OF MOUNT VERNON, NEW YORK.

## METHOD OF TREATING PAPER.

No Drawing.

Application filed June 19, 1923. Serial No. 646,480.

*To all whom it may concern:*

Be it known that I, JUDSON A. DE CEW, a citizen of Canada, residing at Mount Vernon, New York, have invented certain 5 new and useful Improvements in Methods of Treating Paper, of which the following is a specification.

This invention relates to a new process for treating paper making fibres for the 10 purpose of changing the physical character of the fibrous material and rendering it more suitable for high speed machines such as are used in the manufacture of newsprint paper.

15 In the manufacture of newsprint and similar papers in which no rosin size is used, it is still found necessary to use an astringent such as sulphate of alumina, not for the purpose of coagulating sizing material, 20 but for the purpose of rendering the fibres more astringent so that they will not stick to the presses and cause breaks on the machine when running at high speed.

Sulphate of alumina is used in the manu- 25 facture of newsprint paper in the approxi- mate proportions of one part of sulphate of alumina to one hundred parts of paper fibre. As the paper stock passes on the machine, however, it is diluted with water in the 30 proportions of about one part of fibre to about two hundred parts of water, the alum, therefore, will be diluted in the proportions of one part of sulphate of alumina to twenty thousand parts of water. At such a dilu- 35 tion, the sulphate of alumina will be largely decomposed so that the most of the alumina will be taken up by the fibres by absorp- 40 tion and some of the sulphuric acid is also taken into the fibre but the water running away from the machine contains free sul- phuric acid, which will have a tendency to 45 corrode all piping and metallic parts with which it comes in contact, especially when it is used over and over again in the process of manufacture, in which case, the amount of acidity will increase up to a certain point of stability depending upon the amount of 50 fresh water used.

In practice, it is fully recognized that 55 the use of sulphate of alumina in a newsprint paper-mill is a constant source of cor- 60 rosion and wear and tear, both as regards machine piping and also the wires and cot- ton felts of the paper machine.

Up to the present time, no other material

than sulphate of alumina has been found to give the same results, so that the corrosive effect of the alum in these mills is tolerated in order to get machine production.

I have discovered, however, a substitute 60 for sulphate of alumina in this process which will not only have the same similar astringent effects upon the fibres which prevent their sticking to the presses, but it is a chemical and a stronger base and when 65 in solution will not decompose as much as sulphate of alumina and consequently does not produce the free acid which causes corrosion.

The chemical material is not one of the 70 usual soluble salts known to the trade but is material which is known in the trade as an insoluble filling material and is used, at the present time, solely for the purpose of loading papers in order to increase their 75 weight.

The reason it has never been used know- 80 ingly in the solution form as an alum sub- 85 titute is because it is very slightly soluble, its saturated solution containing only two parts per one thousand of water. This ma- terial is the well known filling material, calcium sulphate, ( $\text{CaSO}_4$ ) It would be possible therefore, to dissolve forty pounds of this material in twenty thousand pounds 85 of water so that its solubility is moderately in excess of the amount necessary of its use as a substitute for sulphate of alumina.

My method of using this material is to mix ground or precipitated calcium sulphate 90 with the largest amount of water that can be conveniently added to the paper stock, or it may be added directly into the beaters or mixing chest.

The process is preferably carried in such 95 a manner that when the diluted paper stock passes on the wire it would contain in solu- 100 tion, approximately twenty parts of cal- cium sulphate to one ten thousand of fibrous material.

It is not desirable to obtain a supersatu- 105 rated solution but merely a solution which will act almost in the same way as sulphate of alumina because the fibres will take up a portion of this salt by adsorption which prevents their sticking to the presses and thus all the technical advantages obtained from sulphate of alumina are duplicated.

This salt, however, does not produce 110 acidity in the solution and consequently

there will be no corrosive effect upon any part of the machine or the machine clothing.

This material also had a tendency to harden the pitchy material sometimes found in ground wood and sulphite pulp. It apparently forms a calcium resinate over the surface of the pitch.

Up to the present time, the slight amount of solubility of calcium sulphate has been the chief objection to its use as a filling material and no one has ever claimed that the solution of calcium sulphate could be used to any advantage in paper making.

I therefore claim as my invention:

The process of treating paper-making fibres to be used in a slack sized paper, to render them more astringent, which consists in bringing them into contact before or during the paper-making process with an aqueous solution of calcium sulphate in which there is more calcium sulphate than in natural mill water, but not enough to act as a filler for the paper.

In testimony whereof I have affixed my signature to this specification.

JUDSON A. DE CEW.